# EUROPEAN PATENT SPECIFICATION

(11) **EP 0 729 157 B1**
(45) Date of publication and mention of the grant of the patent: **29.04.1998**
(21) Application number: 95102703.6
(22) Date of filing: 24.02.1995
(51) Int. Cl.: H01B 7/34, H01B 3/10

(54) **Electrical conductor member such as a wire with an inorganic insulating coating**
Elektrisches Leiterelement wie ein Draht mit anorganischen Isolierbeschichtung
Elément électrique conducteur tel qu'un fil muni d'un revêtement isolant inorganique

(43) Date of publication of application: 28.08.1996
(73) Proprietor: SUMITOMO ELECTRIC INDUSTRIES, LTD., Osaka-shi, Osaka 541 (JP)
(72) Inventor: Sawada, Kazuo, c/o Osaka Works of Sumitomo, Konohana-ku, Osaka (JP); Inazawa, Shinji, c/o Osaka Works of Sumitomo, Konohana-ku, Osaka (JP); Yamada, Kouichi, c/o Osaka Works of Sumitomo, Konohana-ku, Osaka (JP)
(74) Representative: Thiel, Christian, Dr. Dipl.-Chem.

(56) References cited:
- EP-A- 0 188 370
- EP-A- 0 292 780
- EP-A- 0 416 131
- EP-A- 0 494 424

## Description

### BACKGROUND OF THE INVENTION

### Field of the Invention

The present invention relates to an electrically conducting wire with an insulating coating made of an inorganic material. Such a wire is used for high temperature operating conditions, e.g. as an insulated lead wire or the like.

### Description of the Background Art

An insulated conductor such as a wire or a member for a thermocouple is generally used in equipment such as heating equipment or fire alarm devices, which require safe operation at high operating temperatures. Such an insulated wire is also employed in an automobile in an environment which is heated to a high temperature. An insulated wire of this type is generally formed by a conductor which is coated with a heat-resistant organic resin such as polyimide, fluororesin or the like.

Such a resin-coated wire can merely withstand a temperature of about 300°C at the most. However, a wire which is employed in a high vacuum apparatus, for example, must have high heat resistance against baking, etc., a small emission characteristic as to absorbed gas and water for achieving and maintaining a high degree of vacuum, and a small emission of gases caused by thermal decomposition. It is impossible to satisfy such requirements for heat resistance and a non-outgassing property with a conventional wire which is coated with an organic material insulation.

When an insulated wire is used where a high heat resistance is required or in an environment requiring a high degree of vacuum, it is impossible to attain a sufficient heat resistance nor the required non-outgassing property with only an organic coating. In that case, therefore, an insulated wire is comprising a conductor which passes through an insulator tube of ceramics, an MI (mineral insulated) cable comprising a conductor which passes through a tube of a heat-resistant alloy, such as stainless steel alloy, that is filled with fine particles of a metal oxide such as magnesium oxide, or the like is generally used.

On the other hand, a glass braided tube insulated wire employing an insulating member of glass fiber fabric or the like is known as an insulated, heat resistant, flexible wire.

Further, wires coated with in organic materials were studied. As a result, wires have been proposed, one of which is obtained by anodizing an aluminum (Aℓ) conductor for forming an Aℓ oxide layer on the outer wire surface, and another wire is obtained by mixing a frit prepared by mixing various metal oxides with each other and melting and pulverizing the as-obtained mixture for forming a slip, applying this slip to a metal conductor and heating and melting the same for forming a homogeneous composite metal oxide layer or coating on the wire surface.

However, the wire with an aluminum oxide layer is not suitable for use as a heat resistant wire since this technique is merely applicable to an aluminum conductor having a low melting point, while the as-formed film is so porous that the wire has an inferior moisture resistance and a low breakdown voltage.

On the other hand, the wire with a composite metal oxide coating is applicable to a metal conductor of copper (Cu) or nickel (Ni) having a higher heat resistance. In practice, however, this technique is merely applicable to a metal composite oxide whose melting point is lower by about 300 to 400°C than those of Cu and Ni since the metal composite oxide layer is formed through a melting process, and the heat resistance temperature is restricted below the just mentioned level. Further, the as-formed wire is inferior in flexibility since it is difficult to reduce the thickness of the film.

In the case of the MI cable, on the other hand, the overall diameter is increased as compared with the conductor diameter, leading to an inferior space factor. Thus, it is impossible to feed a high current.

In the glass braided tube insulated wire, further, fine glass powder is generated and the conductor is disadvantageously exposed due to mesh displacement.

EP-A-0 494 424 discloses Ni or Ni alloy wires having an inner oxide layer of Ni or Ni alloy and an outer insulating inorganic compound layer of SiO₂, Al₂O₃, MgO, ZrO₂ and mixtures thereof.

### SUMMARY OF THE INVENTION

It is an object of the present invention to provide an inorganic insulated member such as an electric conductor wire which has an excellent heat resistance and insulability.

The inorganic insulating member or electrical conductor wire according to the present invention comprises a conductor of Ni or Ni alloy, an oxide layer of an oxide of Ni or Ni alloy on an outer surface of the conductor, said oxide layer being obtained by oxidizing the conductor in a vapor phase containing oxygen, an oxide layer of silicon (Si) on an outer surface of the oxide layer of Ni or Ni alloy, and an oxide layer of aluminum (Al) on an outer surface of the oxide layer of Si.

According to the present invention, the oxide layers of Aℓ and Si are oxide layers obtained by applying a solution prepared by hydrolyzing and polycondensing alkoxide of Aℓ or Si in a solvent, drying the same for allowing gelation, and thereafter heating the obtained gel.

According to the present invention, further, the oxide layers of Aℓ and Si have a melting point exceeding that of Ni or Ni alloy.

The inorganic insulated member according to the present invention is applied to or used as a heat resistant wire or an incombustible wire at a high temperature which does not permit using an organic insulating material, for example. However, the present invention is not restricted to such a wire, but is also applicable to another member such as a thermocouple.

The foregoing and other objects, features, aspects and advantages of the present invention will become more apparent from the following detailed description of the present invention when taken in conjunction with the accompanying drawings.

### BRIEF DESCRIPTION OF THE DRAWINGS

Fig. 1 is a sectional view showing a wire in accordance with present reference example 1 with a nickel conductor core and two oxide layers;
Fig. 2. is a sectional view showing a wire in accordance with present reference example 2 with a nickel alloy core conductor and two oxide layers;
Fig. 3 is a sectional view showing a wire of the present invention with a nickel core conductor and three oxide layers; and
Fig. 4 is a sectional view showing a wire in accordance with present reference example 3 with a nickel alloy core conductor and two oxide layers.

### DESCRIPTION OF THE PREFERRED EMBODIMENTS

Fig. 1 shows an Ni core conductor 1 coated with a Ni oxide layer 2 formed around the core conductor. An Aℓ oxide layer 3 is formed around the Ni oxide layer 2. The formation of these oxide layers will be described in more detail below.

Fig. 2 shows a nickel alloy conductor 11 first coated with a Ni alloy oxide layer 12 formed around the Ni alloy conductor 11. A Si oxide layer 13 is formed around the Ni alloy oxide layer 12.

In Fig. 3 the nickel Ni core conductor 21 is first coated with a Ni oxide layer 22 formed around the Ni core conductor 21. A Si oxide layer 23 is formed around the Ni oxide layer 22. Then, an Aℓ oxide layer 24 is formed around the Si oxide layer 23.

In Fig. 4, a nickel alloy core conductor 31 is first coated with an Ni alloy oxide layer 32 formed around the Ni alloy core conductor 31. Then, an Aℓ-Si composite oxide layer 33 is formed around the Ni alloy oxide layer 32.

According to the present invention, a first oxide layer of Ni or an Ni alloy is first formed on an outer surface of a conductor of Ni or Ni alloy by oxidizing the conductor in a vapor phase containing oxygen. Then, a second oxide layer of Si is formed on the first oxide layer.

Ni or Ni alloy is an inactive metal which has an inferior affinity for a metal oxide of Aℓ or Si. When a surface of Ni or Ni alloy is directly coated with such an Aℓ or Si oxide, a rather poor adhesion is obtained and the coating is immediately separated from the Ni or Ni alloy. In order to solve this problem, the present invention teaches to first oxidize a core conductor of Ni or Ni alloy in a vapor phase containing oxygen, so as to form an oxide layer of Ni or Ni alloy. The so formed nickel oxide layer or Ni alloy oxide layer very strongly adheres to the surface of the Ni or Ni alloy. This strong bonding is due to the fact that the nickel oxide or the nickel alloy oxide has an excellent affinity for the nickel or nickel alloy. Additionally, the nickel or nickel alloy oxide has a strong affinity to silicon oxide and hence also strongly bonds to the outer layer of Si oxide and to the conductor core. According to the present invention, therefore, the oxide layer of Si is not separated for all practical purposes from the intermediate oxide layer, whereby an excellent flexibility is obtained when the inorganic insulating coating is applied to a wire forming a core conductor, for example.

According to the present invention, the oxide layers of Aℓ and Si are obtained by applying a solution prepared by hydrolyzing and polycondensing an alkoxide of Aℓ or Si in a solvent, drying the same for allowing gelation, and thereafter heating the so-obtained gel.

The Aℓ and Si oxide layers formed in the aforementioned manner have a melting point exceeding that of the Ni or Ni alloy. Additionally, the Aℓ and Si oxide layers are formed without any melting process.

Therefore, the critical temperature to which conductors or other members of the present invention with their inorganic insulating coatings may be exposed in operation is not restricted by the melting point of the oxide layer. Rather, the present insulating members can be heated to a temperature limited only by the melting point of the Ni core or the Ni alloy core.

Further, the oxide layer formed in the aforementioned manner has characteristics such as an extreme denseness, a smooth surface and a small adsorption of gases, e.g. steam or the like. Moreover, the present members have an excellent insulability and a high moisture resistance.

Preferred embodiments have been produced as two conductors C1 and C2 which were oxidized as follows.
(C1) An Ni wire of 0.5 mm is diameter consisting of at least 99.9 % by weight of Ni, the remainder being natural impurities was heated in the atmosphere at 950°C for 10 minutes, to form a nickel oxide layer on the surface of the wire.
(C2) An Ni alloy wire of 0.5 mm in diameter containing 15 % by weight of Cr was heated in the atmosphere at 850°C for 30 minutes, to form an oxide layer of Ni alloy on the wire surface.

The following coating solutions L1, L2 and L3 were prepared as follows:
(L1) A solution L1 was obtained by mixing tributoxy aluminum, triethanolamine, water, and isopropyl alcohol in mole ratios of 1:2:1:16. The mixture was hydrolyzed and polycondensed at 50°C for 1 hour while stirring the mixture.
(L2) A solution L2 was obtained by adding nitric acid to a mixed solution prepared by mixing tributyl orthosilicate, water, and isopropyl alcohol in mole ratios of 2:8:15 at a rate of 3/100 moles with respect to tetrabutyl orthosilicate. The mixture was hydrolyzed and polycondensed at 80°C for 2 hours while stirring the mixture.
(L3) A solution L3 was obtained by mixing the solutions L1 and L2 at a mass ratio of 80:20.

Reference Example 1: An oxidized nickel conductor C1 was coated with the coating solution L1 and heated at 500°C for 10 minutes. The coating and heating was repeated 10 times, to form an Aℓ oxide layer of 4 µm thickness on the first nickel oxide layer.

Reference Example 2: An oxidized nickel alloy conductor C2 was coated with the coating solution L2 and heated at 500°C for 10 minutes. The coating and heating was repeated 10 times, to form a Si oxide layer of 5 µm thickness on the first nickel alloy oxide layer.

Example 1: An oxidized nickel conductor C1 was coated with the coating solution L2 and heated at 500°C for 10 minutes.

The coating and heating was repeated 5 times to form a Si-oxide layer having a thickness of 2.5 µm. Then, a further coating operation was performed on the first formed Si-oxide layer, with the coating solution L1. The sample was again heated at 500°C for 10 minutes. The coating and heating was repeated 5 times to form an Aℓ oxide layer of 2 µm thickness on the first formed Si oxide layer of 2.5 µm thickness.

Reference Example 3: An oxidized conductor C2 was coated with the coating solution L3 and heated at 500°C for 10 minutes. The coating and heating was repeated 10 times to form an Aℓ-Si composite oxide layer of 6 µm in thickness.

Comparative Example 1: An aluminum wire was anodized in a bath of sulfuric acid to form an Aℓ oxide layer of 10µm thickness on the aluminum surface.

Comparative Example 2: An oxidized conductor C2 was coated-with a slip which was prepared by mixing a commercially available frit (composite oxide of Ba, Ca, Ti and Si: GSP220A552 sold by Toshiba Glass Co., Ltd.) with water. The wire coated with the slip was heated to 900°C to form a homogenous metal composite oxide layer of 100 µm thickness through a melted state.

All the coating operations were, for example, performed by dipping the wire into the respective coating solution.

### Test Results

| Example | Breakdown Voltage | Flexibility |
|---|---|---|
| Reference Example 1 | 500 V | 6D |
| Reference Example 2 | 600 V | 5D |
| 1 | 800 V | 8D |
| Reference Example 3 | 400 V | 3D |
| Comparative Example 1 | 300 V | 50D |
| Comparative Example 2 | 1200 V | 1000D |

The above Table shows the breakdown voltages and the flexibility values of the wires of Example 1 of the invention, of Reference Examples 1 to 3 and of the two Comparative Examples. The flexibility values were evaluated in terms of diameter ratios, by winding the wires on circular cylinders of a prescribed diameter D and measuring the minimum diameters causing no separation of the insulating inorganic compound coatings or layers from the conductor core. The diameter D was 0.5 mm.

The above Table shows that the wire of Example 1 according to the present invention has a higher breakdown voltage than the first Comparative Example and a superior flexibility compared to both Comparative Examples. However, the second Comparative Example has a substantially higher breakdown voltage at the expense of being very stiff.

As hereinabove described, the inorganic insulating coating on a conductor wire according to the present invention forms an insulating inorganic compound layer which is well bonded to the conductor core and has an excellent heat resistance and insulability.

Although the present invention has been described and illustrated in detail, it is clearly understood that the same is by way of illustration and example only and is not to be taken by way of limitation, the scope of the present invention being limited only by the terms of the appended claims.

## Claims

1. An insulated electrical conductor comprising a core conductor (21) consisting essentially of a core material selected from the group consisting of Ni and Ni alloy, a first oxide layer (22) consisting of an oxide of said core material formed on an outer surface of said core conductor (21) by oxidizing said core conductor in a vapor phase containing oxygen, and a second oxide layer (23) bonded to an outer surface of said first oxide layer, said second oxide layer consisting essentially of Si-oxide, characterized by further comprising a third oxide layer (24) on an outer surface of said second oxide layer (23), said third oxide layer (24) consisting essentially of Al-oxide.

2. The insulated electrical conductor according to claim 1, wherein said second oxide layer (23) has a melting temperature greater than that of said core material (21).

3. The insulated electrical conductor according to claim 1, wherein said core conductor (21) consists of Ni and trace amounts of naturally occurring impurities.

4. The insulated electrical conductor according to claim 1, wherein said core conductor (21) consists essentially of Ni and Cr.

5. The insulated electrical conductor according to claim 4, wherein said core conductor (21) consists essentially of about 85 % Ni and about 15 % Cr.

6. A method of forming an insulated electrical conductor, comprising:
(a) preparing a core conductor (21) of a core material selected from the group consisting of Ni and Ni alloy;
(b) forming a first oxide layer (22) on an outer surface of said core conductor (21) by oxidizing said core conductor in a vapor phase containing oxygen;
(c) preparing a first coating solution by hydrolyzing and polycondensing an alkoxide of Si in a solvent;
(d) applying said first coating solution onto said first oxide layer (22);
(e) drying said first coating solution for gelling the same; and
(f) heating said first coating solution applied onto said first oxide layer (22) to form a second oxide layer (23) on said oxide layer;
characterized by further comprising:
(g) preparing a second coating solution by hydrolyzing and polycondensing an alkoxide of Al in a solvent;
(h) applying said second coating solution onto said second oxide layer (23); and
(i) heating said second coating solution to form a third oxide layer (24) on said second oxide layer (23).

7. The method of claim 6, further comprising repeating said steps (d) to (f) and/or (g) to (i) a plurality of times, whereby successive coating films of said coating solution are applied one on top of another to form said second and third oxide layers (22, 23).

8. The method of claim 6, wherein said step (f) does not involve a melting process.

9. The method of claim 6, wherein said second coating solution is prepared by forming a mixture of tributoxy aluminum, triethanolamine, water and isopropyl alcohol, and then hydrolyzing and polycondensing said mixture.

10. The method of claim 9, wherein the respective mole ratio of said tributoxy aluminum, triethanolamine, water and isopropyl alcohol is 1:2:1:16, and said hydrolyzing and polycondensing is carried out at 50°C for 1 hour while stirring said mixture.

11. The method of claim 6, wherein said first coating solution is prepared by forming a mixture of tributyl orthosilicate, water and isopropyl alcohol, adding nitric acid to said mixture, and then hydrolyzing and polycondensing said mixture with said nitric acid added thereto.

12. The method of claim 11, wherein the respective mole ratio of said tributyl orthosilicate, water and isopropyl alcohol is 2:8:15, said nitric acid is added at a rate of 3/100 moles with respect to tributyl orthosilicate, and said hydrolyzing and polycondensing is carried out at 80°C for 2 hours while stirring said mixture.

13. The method of claim 6, wherein said heating step is carried out at about 500°C.

## Patentansprüche

1. Isolierter elektrischer Leiter, umfassend einen Kernleiter (21), bestehend im wesentlichen aus einem Kernmaterial, ausgewählt aus der Gruppe, bestehend aus Ni und Ni-Legierung, eine erste Oxidschicht (22), bestehend aus einem Oxid des Kernmaterials, die auf einer äußeren Oberfläche das Kernleiters (21) durch Oxidieren des Kernleiters in einer Sauerstoff enthaltenden Dampfphase erzeugt worden ist, und eine zweite Oxidschicht (23), die an eine äußere Oberfläche der ersten Oxidschicht gebunden ist, wobei die zweite Oxidschicht im wesentlichen aus Si-Oxid besteht, dadurch gekennzeichnet, daß er zusätzlich eine dritte Oxidschicht (24) auf einer äußeren Oberfläche der zweiten Oxidschicht (23) umfaßt, wobei die dritte Oxidschicht (24) im wesentlichen aus Al-Oxid besteht.

2. Isolierter elektrischer Leiter nach Anspruch 1, wobei die zweite Oxidschicht (23) eine Schmelztemperatur besitzt, die höher liegt als diejenige des Kernmaterials (21).

3. Isolierter elektrischer Leiter nach Anspruch 1, wobei der Kernleiter (21) aus Ni und Spurenmengen von natürlich vorkommenden Verunreinigungen besteht.

4. Isolierter elektrischer Leiter nach Anspruch 1, wobei der Kernleiter (21) im wesentlichen aus Ni und Cr besteht.

5. Isolierter elektrischer Leiter nach Anspruch 4, wobei der Kernleiter (21) im wesentlichen aus etwa 85% Ni und etwa 15% Cr besteht.

6. Verfahren zur Herstellung eines isolierten elektrischen Leiters, umfassend:
(a) Herstellen eines Kernleiters (21) aus einem Kernmaterial, ausgewählt aus der Gruppe, bestehend aus Ni und Ni-Legierung;
(b) Erzeugen einer ersten Oxidschicht (22) auf einer äußeren Oberfläche das Kernleiters (21) durch Oxidieren des Kernleiters in einer Sauerstoff enthaltenden Dampfphase;
(c) Herstellen einer ersten Überzugslösung durch Hydrolysieren und Polykondensieren eines Alkoxids von Si in einem Lösungsmittel;
(d) Aufbringen der ersten Überzugslösung auf die erste Oxidschicht (22);
(e) Trocknen der ersten Überzugslösung. um sie zur Gelbildung zu bringen;
(f) Erhitzen der auf die erste Oxidschicht (22) aufgebrachten ersten Überzugslösung zur Bildung einer zweiten Oxidschicht (23) auf der Oxidschicht,
dadurch gekennzeichnet, daß es ferner umfaßt:
(g) Herstellen einer zweiten Überzugslösung durch Hydrolysieren und Polykondensieren eines Alkoxids von Al in einem Lösungsmittel;
(h) Aufbringen der zweiten Überzugslösung auf die zweite Oxidschicht (23) und
(i) Erhitzen der zweiten Überzugslösung zur Bildung einer dritten Oxidschicht (24) auf der zweiten Oxidschicht (23).

7. Verfahren nach Anspruch 6, umfassend ferner das mehrmalige Wiederholen der Stufen (d) bis (f) und/oder (g) bis (i), wodurch aufeinanderfolgende Überzugsfilme aus der Überzugslösung übereinander aufgebracht werden zur Bildung der zweiten und dritten Oxidschichten (23, 24).

8. Verfahren nach Anspruch 6, wobei die Stufe (f) keinen Schmelzprozeß umfaßt.

9. Verfahren nach Anspruch 6, wobei die zweite Überzugslösung hergestellt wird durch Bilden eines Gemisches aus Tributoxyaluminium, Triethanolamin, Wasser und Isopropylalkohol und anschließendes Hydrolysieren und Polykondensieren des Gemisches.

10. Verfahren nach Anspruch 9, wobei das jeweilige Molverhältnis von dem Tributoxyaluminium, Triethanolamin, Wasser und Isopropylalkohol 1:2:1:16 beträgt und das Hydrolysieren und Polykondensieren 1 Stunde bei 50°C unter Rühren des Gemisches durchgeführt wird.

11. Verfahren nach Anspruch 6, wobei die erste Überzugslösung hergestellt wird durch Bilden eines Gemisches aus Tributylorthosilicat, Wasser und Isopropylalkohol, Zugeben von Salpetersäure zu dem Gemisch und anschließendes Hydrolysieren und Polykondensieren des Gemisches mit der zugesetzten Salpetersäure.

12. Verfahren nach Anspruch 11, wobei das jeweilige Molverhältnis von dem Tributylorthosilicat, Wasser und Isopropylalkohol 2:8:15 beträgt, die Salpetersäure in einer Menge von 3/100 Mol, bezogen auf das Tributylorthosilicat, zugegeben wird und das Hydrolysieren und Polykondensieren 2 Stunden bei 80°C unter Rühren des Gemisches durchgeführt wird.

13. Verfahren nach Anspruch 6, wobei die Stufe des Erhitzens bei etwa 500°C durchgeführt wird.

## Revendications

1. Conducteur électrique isolé comprenant une âme conductrice (21) constituée essentiellement d'un matériau d'âme choisi parmi le groupe constitué de Ni et d'alliage de Ni, une première couche d'oxyde (22) constituée d'un oxyde dudit matériau d'âme, formée sur une surface extérieure de ladite âme conductrice (21) en oxydant ladite âme conductrice dans une phase vapeur contenant de l'oxygène, et une seconde couche d'oxyde (23) liée à une surface extérieure de ladite première couche d'oxyde, ladite seconde couche d'oxyde étant constituée essentiellement d'oxyde de Si, caractérisé en ce qu'il comprend en outre une troisième couche d'oxyde (24) sur une surface extérieure de ladite seconde couche d'oxyde (23), ladite troisième couche d'oxyde (24) étant essentiellement constituée d'oxyde d'Al.

2. Conducteur électrique isolé selon la revendication 1, dans lequel ladite seconde couche d'oxyde (23) a une température de fusion supérieure à celle dudit matériau d'âme.

3. Conducteur électrique isolé selon la revendication 1, dans lequel ladite âme conductrice (21) est constituée de Ni et de traces d'impuretés d'origine naturelle.

4. Conducteur électrique isolé selon la revendication 1, dans lequel ladite âme conductrice (21) est constituée essentiellement de Ni et Cr.

5. Conducteur électrique isolé selon la revendication 4, dans lequel ladite âme conductrice (21) est constituée essentiellement d'environ 85% de Ni et d'environ 15% de Cr.

6. Procédé de formation d'un conducteur électrique isolé, comprenant :
(a) la préparation d'une âme conductrice (21) en un matériau d'âme choisi parmi le groupe constitué de Ni et d'alliage de Ni ;
(b) la formation d'une première couche d'oxyde (22) sur une surface extérieure de ladite âme conductrice (21) en oxydant ladite âme conductrice dans une phase vapeur contenant de l'oxygène ;
(c) la préparation d'une première solution de revêtement, en hydrolysant et en polycondensant un alcoxyde de Si dans un solvant ;
(d) l'application de ladite première solution de revêtement sur ladite première couche d'oxyde (22) ;
(e) le séchage de ladite première solution de revêtement pour gélifier celle-ci ; et
(f) le chauffage de ladite première solution de revêtement appliquée sur ladite première couche d'oxyde (22) pour former une seconde couche d'oxyde (23) sur ladite couche d'oxyde ;
caractérisé en ce qu'il comprend en outre :
(g) la préparation d'une seconde solution de revêtement en hydrolysant et en polycondensant un alcoxyde de Al dans un solvant ;
(h) l'application de ladite seconde solution de revêtement sur ladite seconde couche d'oxyde (23) ; et
(i) le chauffage de ladite seconde solution de revêtement pour former une troisième couche d'oxyde (24) sur ladite seconde couche d'oxyde (23).

7. Procédé selon la revendication 6, comprenant en outre la répétition desdites étapes (d) à (f) et/ou (g) à (i) plusieurs fois, grâce à quoi des films de revêtement successifs de ladite solution de revêtement sont appliqués l'un au dessus de l'autre, pour former lesdites seconde et troisième couches d'oxyde (22, 23).

8. Procédé selon la revendication 6, dans lequel ladite étape (f) ne nécessite pas un procédé de fusion.

9. Procédé selon la revendication 6, dans lequel ladite seconde solution de revêtement est préparée en formant un mélange de tributoxyaluminium, de triéthanolamine, d'eau et d'alcool isopropylique, et ensuite en hydrolysant et en polycondensant ledit mélange.

10. Procédé selon la revendication 9, dans lequel le rapport molaire respectif desdits tributoxyaluminium, triéthanolamine, eau et alcool isopropylique est 1:2:1:16, et lesdites hydrolyse et polycondensation sont effectuées à 50°C, pendant 1 heure, tout en agitant ledit mélange.

11. Procédé selon la revendication 6, dans lequel ladite première solution de revêtement est préparée en formant un mélange d'orthosilicate de tributyle, d'eau et d'alcool isopropylique, en ajoutant de l'acide nitrique audit mélange, et ensuite en hydrolysant et en polycondensant ledit mélange avec ledit acide nitrique qui y a été ajouté.

12. Procédé selon la revendication 11, dans lequel le rapport molaire respectif desdits orthosilicate de tributyle, eau et alcool isopropylique est 2:8:15, ledit acide nitrique est ajouté à un taux de 3/100 moles par rapport à l'orthosilicate de tributyle, et lesdites hydrolyse et polycondensation sont effectuées à 80°C, pendant 2 heures, tout en agitant ledit mélange.

13. Procédé selon la revendication 6, dans lequel ladite étape de chauffage est effectuée à environ 500°C.
